

## UNITED STATES PATENT OFFICE

2,235,243

FERROUS METAL ARTICLE AND METHOD OF  
PRODUCING SAME

Joseph S. Adelson, Shaker Heights, Ohio, assignor,  
by mesne assignments, to Republic Steel Corporation,  
Cleveland, Ohio, a corporation of New Jersey

No Drawing. Application March 27, 1939,  
Serial No. 264,483

10 Claims. (Cl. 148—12)

This invention relates to the art of making ferrous metal articles, and is particularly concerned with articles, such as tube and pipe, which are composed of the less expensive steel compositions and yet possess new and improved physical properties, and is also concerned with a new and improved method for producing such articles.

The physical properties obtained in ferrous metal articles heretofore were determined largely by the size and composition of the articles. For example, a steel composition was usually selected which would give the desired physical properties in an article of given dimensions. Where the physical properties desired were higher than those obtainable with an inexpensive steel composition within the specified dimensions, a more expensive composition was usually employed, i. e., one containing one or more alloying ingredients which would give to the steel the higher properties desired. For some time the tendency has been to demand higher and higher physical properties and, as a result, more and more expensive compositions have been used in producing such articles, and this tendency has been particularly noticeable in the tube and pipe field. Since the cost of the steel used is a large part of the cost of the article, the use of the more expensive steel compositions has considerably increased the cost of manufacture of the articles, and this has been especially true in the tube and pipe field where the demand for higher physical properties has been pronounced.

The present invention aims to use the less expensive steel compositions and yet to produce articles made therefrom which will have improved physical properties corresponding to those of articles having greater dimensions or composed of more expensive steel compositions. Briefly, I attain these objects by selecting a ferrous metal composition having physical properties which, in an article of the desired dimensions or in an article of thinner wall thickness, will be somewhat lower than those required in the article and then, by suitably cold working and heat treating the metal, improving the physical properties so that the resulting article will have the required physical properties. In other words, this invention makes it possible to use a lower grade of steel or a smaller amount of the same grade of steel and still obtain the required physical properties in the final article. This makes it possible to lower the cost by using a less expensive metal or to decrease the weight by using a smaller amount of metal. Often both cost and weight may be decreased.

The present invention is applicable to ferrous metal of many different compositions. For example, it is applicable to the class of steels known as simple or low carbon steels, which class is illustrated by the steel which is known commercially as SAE-1020 and which contains between about .15% and about .25% of carbon, and between about .30% and about .60% of manganese, the remainder being iron with the usual amounts of ordinary impurities. It is also applicable to the class of steels known generally as alloy steels. This class includes steels containing between about .10% and about .35% of carbon, between about .30% and about 1.5% of manganese, one or more of the metals copper, chromium and nickel in amounts up to about 1.5% and/or molybdenum up to about .40%, the remainder of the composition being iron with the usual amounts of ordinary impurities. It will be understood that when more than one of these additional metals are present, the total amount of such metals should not exceed about 1.5%. It is also applicable to steels whose compositions lie between the two foregoing classes.

The present invention is also applicable to steels containing carbon in excess of about .35% for uses where improved yield points and tensile strengths are desired, and where somewhat decreased ductility and increased hardness and brittleness are not detrimental.

The present process consists, as indicated above, of the two major steps of cold working and heat treating. The cold working step may be carried out on the metal when it is in hot rolled, or cold rolled and annealed, strip form, as by cold rolling the strip before it is formed into an article of the desired shape, for example a tube or pipe; or the hot rolled, or cold rolled and annealed, strip may be formed into an article, such as a tube or pipe, and welded and then cold worked to the desired extent, as by cold drawing the article; or the hot rolled strip may be cold worked by rolling and the article made therefrom may be further cold worked if desired, as by drawing.

In making tube or pipe by this invention, any standard method of welding may be employed but, since the electric resistance butt welding method is rapid, economical and comparatively inexpensive, I prefer to employ that method.

The second major step of the process, that is the heat treating of the article composed of cold worked metal, may be carried out by heating the article at a temperature of between about 500° F. and between about 850° F., for a length of time

dependent on the thickness of the steel, the time being determined at the rate of about one minute for each  $\frac{1}{30}$ " to  $\frac{1}{60}$ " of metal thickness, or, in other words, at the rate of an hour for 2" to 5 1" of metal thickness. Then the article is allowed to cool in the air.

I have found that when the steel is cold worked to an extent equivalent to a cold reduction in thickness of between about 10% and about 25%, 10 and is thereafter heat treated, as described, the yield point may be increased from about 10% to about 25%, the tensile strength may be increased from about 5% to about 20% and the increase in elongation in 2" may amount to as much as 15 about 50%.

The following examples are illustrative of the results obtainable by use of the present process:

Cold rolled, annealed, 21 gage, SAE-1020, strip steel containing about .20% of carbon, about 20 .50% of manganese, the remainder being iron with the usual amounts of ordinary impurities was formed and electric resistance butt welded into a tube 1 $\frac{1}{8}$ " in outside diameter. This strip might be considered as being a "soft strip" because it was annealed after cold rolling which had the effect of reducing or largely eliminating the increase in physical properties which had been given to it by the cold rolling operation. The welded tube was cold drawn to 1" O. D., 25 which cold worked it in an amount equivalent to a cold reduction in thickness of between about 10% and about 25%, and then the tube was heated at about 750° F. for about 2 minutes and allowed to cool in the air. The physical properties of the resulting tube, after welding, after drawing and after heat treatment are set out in the following table:

| 40            | Condition when tested | Minimum yield point      | Minimum tensile str.     | Minimum percent elong. in 2" |
|---------------|-----------------------|--------------------------|--------------------------|------------------------------|
|               |                       | lb. per sq. in. of metal | lb. per sq. in. of metal | of metal                     |
| As welded     |                       | 50,000                   | 60,000                   | 25                           |
| After drawing |                       | 60,000                   | 70,000                   | 15                           |
| 45            | After heat treatment  | 70,000                   | 80,000                   | 15                           |

Another strip of SAE-1020 steel having substantially the same composition as that given hereinabove was cold rolled, formed and welded into tube and then heat treated. The strip was cold worked to an extent equivalent to a cold reduction in thickness of about 18%. This strip might be considered as "cold worked strip" in contrast to the "soft strip" of the preceding example. The results in the as welded and heat treated conditions were as follows:

| 60         | Treatment | Yield point               | Tensile str.              | Elongation               |
|------------|-----------|---------------------------|---------------------------|--------------------------|
|            |           | lbs. per sq. in. of metal | lbs. per sq. in. of metal | in 2" — percent of metal |
| As weld    |           | 70,900                    | 76,800                    | 16                       |
| Do.        |           | 73,000                    | 79,100                    | 24                       |
| 750° H. T. |           | 77,800                    | 82,200                    | 17                       |
| Do.        |           | 76,800                    | 82,800                    | 25                       |

65 Another steel containing about .18% of carbon, about 1.00% of manganese and about .90% of copper, the remainder being iron with ordinary amounts of the usual impurities was cold rolled to 18, 19, 20 and 21 gage and annealed. 70 These strips were then cold formed into tube blanks with longitudinal seam edges which were electric resistance butt welded to make tubes of different outside diameters. These tubes were cold drawn to smaller diameters and were then 75 heat treated at about 750° F. The following

results were obtained from such tubes in the drawn and heat treated conditions:

| Condition when tested                                            | Yield point<br>lb. per sq. in.<br>of metal | Tensile str.<br>lb. per sq. in.<br>of metal | Percent<br>elong.<br>in 2" | 5  |
|------------------------------------------------------------------|--------------------------------------------|---------------------------------------------|----------------------------|----|
| 1 $\frac{1}{4}$ " x 18 gage drawn to 1 $\frac{1}{8}$ " x 18 gage | 65,800                                     | 75,000                                      | 19                         |    |
| After heat treatment                                             | 75,700                                     | 79,600                                      | 19                         |    |
| 1 $\frac{1}{4}$ " x 19 gage drawn to 1 $\frac{1}{8}$ " x 19 gage | 67,200                                     | 77,900                                      | 18                         | 10 |
| After heat treatment                                             | 76,600                                     | 83,200                                      | 20                         |    |
| 1 $\frac{1}{4}$ " x 20 gage drawn to 1" x 20 gage                | 68,800                                     | 79,500                                      | 18                         |    |
| After heat treatment                                             | 75,400                                     | 84,600                                      | 17                         |    |
| 1 $\frac{1}{4}$ " x 21 gage drawn to 1" x 21 gage                | 73,100                                     | 80,500                                      | 17                         |    |
| After heat treatment                                             | 81,600                                     | 86,800                                      | 17                         | 15 |

I have found that the cold working which takes place during the forming of steel from sheet or strip into tube or pipe blanks, preliminary to welding, is sufficient to give improved physical properties when heat treated according to this invention. In other words, steel which has been cold rolled and box annealed, may be improved by cold forming the metal into tube or pipe blanks and heat treating it as herein specified after the welding operation. The following results were obtained by using cold rolled and box annealed strip steel in various gages and composed of about .18% carbon, about .90% manganese, about .39% copper, the remainder being iron with the usual amounts of ordinary impurities. This strip was cold formed and welded into tubes of different sizes and, after welding, the tubes were heat treated at about 750° F. as above described, with the following results:

| Size                 | Treatment | Yield point<br>lbs. per sq. in.<br>of metal | Tensile str.<br>lbs. per sq. in.<br>of metal |    |
|----------------------|-----------|---------------------------------------------|----------------------------------------------|----|
| 1 $\frac{1}{4}$ x 18 | Strip     | 33,500                                      | 58,200                                       | 40 |
| 1 $\frac{1}{4}$ x 18 | As welded | 55,550                                      | 60,900                                       |    |
| 1 $\frac{1}{4}$ x 18 | 750°      | 59,400                                      | 67,600                                       |    |
| 1 $\frac{1}{4}$ x 19 | Strip     | 38,500                                      | 62,800                                       |    |
| 1 $\frac{1}{4}$ x 19 | As welded | 59,100                                      | 62,000                                       |    |
| 1 $\frac{1}{4}$ x 19 | 750°      | 69,800                                      | 67,800                                       |    |
| 1 $\frac{1}{4}$ x 20 | Strip     | 38,600                                      | 62,200                                       |    |
| 1 $\frac{1}{4}$ x 20 | As welded | 57,800                                      | 63,900                                       |    |
| 1 $\frac{1}{4}$ x 20 | 750°      | 63,100                                      | 72,500                                       |    |
| 1 $\frac{1}{4}$ x 21 | Strip     | 37,200                                      | 61,300                                       |    |
| 1 $\frac{1}{4}$ x 21 | As welded | 60,000                                      | 65,600                                       |    |
| 1 $\frac{1}{4}$ x 21 | 750°      | 65,500                                      | 73,100                                       | 50 |

The present invention may also be applied to advantage to tubing made from hot rolled metal. Steel composed of about .22% of carbon, about 1.20% of manganese, about .015% of phosphorus, about .029% of sulfur, about 1.04% of copper, the remainder being iron with usual amounts of ordinary impurities was hot rolled to a thickness of .200" and was then cold formed and welded into tubes three inches in outside diameter. The following table gives the properties of such tubes as welded and after being heat treated at 750° F. as described hereinabove:

| Treatment | Yield point<br>lbs. per sq. in.<br>of metal | Tensile str.<br>lbs. per sq. in.<br>of metal | Elongation<br>in 2", per<br>cent | 65 |
|-----------|---------------------------------------------|----------------------------------------------|----------------------------------|----|
| As welded | 55,080                                      | 88,100                                       | 37                               |    |
| 750° F.   | 88,890                                      | 99,000                                       | 37                               |    |
| As welded | 89,520                                      | 93,840                                       | 26                               | 70 |
| 750° F.   | 93,320                                      | 102,600                                      | 34                               |    |

Having thus described the present invention so that those skilled in the art may be able to understand and practice the same, I state that 75

what I desire to secure by Letters Patent is defined in what is claimed.

What is claimed is:

1. The method of making a steel article having improved physical properties which comprises the steps of making an article composed of a pearlitic steel containing from about .10% to about .35% of carbon which has been cold worked to an extent equivalent to a cold reduction of its thickness of between at least 10% and about 50%, and heating an article composed of such cold worked metal at a temperature between about 500° F., and about 850° F., for a length of time equal to about one minute for each  $\frac{1}{30}$ " to  $\frac{1}{60}$ " in wall thickness of said article.
2. The method of making a steel article having improved physical properties which comprises the steps of cold working a pearlitic steel containing from about .10% to about .35% of carbon and thereby reducing its thickness between at least 10% and about 50%, converting the cold rolled steel into an article, and heat treating said article at a temperature between about 500° F., and about 850° F., for a length of time equal to about one minute for each  $\frac{1}{30}$ " to  $\frac{1}{60}$ " of wall thickness of said article.
3. The method of making a steel article having improved physical properties which comprises the steps of cold rolling a pearlitic steel containing from about .10% to about .35% of carbon, annealing the cold rolled steel, converting the steel into an article, heating the article at a temperature between about 500° F., and about 850° F., for a length of time equal to one minute for each  $\frac{1}{30}$ " to  $\frac{1}{60}$ " in wall thickness of the article, and between the annealing and heating steps cold working the metal to an extent equivalent to a cold reduction in thickness of the metal of between at least 10% and about 50%.
4. The method of making a tubular steel article having improved physical properties which comprises the steps of cold working pearlitic steel in sheet or strip form and containing from about .10% to about .35% of carbon and making it into a welded tubular article, heating said article at a temperature between about 500° F., and about 850° F., for a length of time equal to one minute for each  $\frac{1}{30}$ " to  $\frac{1}{60}$ " in wall thickness of said tube, and cold working the metal so that when it is subjected to said heating step it is in a condition equivalent to that produced by a cold reduction in thickness of between at least 10% and about 50%.
5. The method of making a tubular steel article having improved physical properties which comprises the steps of cold working pearlitic steel in sheet or strip form and containing from about .10% to about .35% of carbon to an extent equivalent to a cold reduction in its thickness of between at least 10% and about 50%, making a welded tubular article from such metal, and heating said welded article at a temperature between about 500° F., and about 850° F., for a length of time equal to one minute for each  $\frac{1}{30}$ " to  $\frac{1}{60}$ " in wall thickness thereof.
6. The method of making a tubular steel article having improved physical properties which comprises the steps of cold forming pearlitic steel in strip or sheet form and containing from

about .10% to about .35% of carbon into a tubular blank having longitudinal seam edges and thereby cold working it to an extent equivalent to a cold reduction in wall thickness of between at least 10% and about 50%, welding said edges together to make a tubular article, and heating said welded article at a temperature between about 500° F., and about 850° F., for a length of time equal to one minute for each  $\frac{1}{30}$ " to  $\frac{1}{60}$ " in wall thickness.

7. The method of making a tubular steel article having improved physical properties which includes the steps of cold rolling pearlitic steel in sheet or strip form and containing from about .10% to about .35% of carbon and forming said metal into tubular shape with longitudinal seam edges, the rolling and forming steps cold working the metal to an extent equivalent to a cold reduction in its wall thickness of between at least 10% and about 50%, welding said edges together, and heating said welded tube at a temperature between about 650° F. and about 850° F. for a length of time equal to one minute for each  $\frac{1}{60}$ " in wall thickness thereof.

8. The method of making a tubular steel article having improved physical properties which comprises the steps of cold rolling pearlitic steel in sheet or strip form and containing from about .10% to about .35% of carbon, annealing such cold rolled steel, forming such annealed steel into a tubular blank having longitudinal seam edges and thereby cold working said annealed steel to an extent equivalent to a cold reduction in thickness of between at least 10% and about 50%, welding said edges together to form a welded tubular article, and heating said article at a temperature between about 500° F. and 850° F. for a length of time equal to one minute for each  $\frac{1}{30}$ " to  $\frac{1}{60}$ " in wall thickness thereof.

9. The method of making a tubular steel article having improved physical properties which comprises the steps of cold rolling pearlitic steel in sheet or strip form and containing from about .10% to about .35% of carbon, annealing such cold rolled steel, forming such annealed steel into a tubular blank with longitudinal seam edges, welding said edges together to form a tubular article, cold drawing said welded article and thereby cold working it to an extent equivalent to a cold reduction in its wall thickness of between at least 10% and about 50%, and heating the drawn article at a temperature of between about 500° F. and about 850° F. for a length of time equal to one minute to each  $\frac{1}{30}$ " to  $\frac{1}{60}$ " in wall thickness thereof.

10. The method of making steel tube or pipe having improved physical properties which comprises the steps of working pearlitic sheet or strip steel containing from about .10% to about .35% of carbon and making it into a welded tubular article, cold drawing said article and thereby reducing its wall thickness between at least 10% and about 50%, and heating such drawn article at a temperature between about 500° F., and about 850° F., for a length of time equal to one minute for each  $\frac{1}{30}$ " to  $\frac{1}{60}$ " in wall thickness of said tube.

JOSEPH S. ADELSON.